

July 27, 1937.

H. I. WATERMAN

2,088,500

ACETYLENATION OF MINERAL OILS

Filed April 20, 1935



Inventor: Hein Israel Waterman

By his Attorney: D. A. [Signature]

## UNITED STATES PATENT OFFICE

2,088,500

## ACETYLENIZATION OF MINERAL OILS

Hein Israel Waterman, Delft, Netherlands, assignor to Shell Development Company, San Francisco, Calif., a corporation of Delaware

Application April 20, 1935, Serial No. 17,492  
In the Netherlands April 23, 1934

5 Claims. (Cl. 196—78)

My process relates to the treatment of mineral oils with acetylene in the presence of aluminum chloride or other suitable catalysts. In particular it deals with the treatment of mineral oils containing aromatics, and with the production of valuable products therefrom.

It is a purpose of my invention to provide a method whereby stocks of relatively low value can be converted into valuable and useful products. For instance, my method enables the production of refined smokeless kerosenes, high viscosity index lubricating oils, resinous products suitable for paints and varnishes, plastic masses adaptable for moldings, drying oils, etc., from cracked fuels and similar low grade hydrocarbon oils. Furthermore, undesirable sulfur compounds are removed.

Suitable treating stocks are crude oils containing aromatics such as are found in Borneo and California, or distillates or residues therefrom; cracked products, in particular residues from cracking operations; Edeleanu extracts or extracts from other solvent extraction processes; liquid products obtained from thermal treatment of hydrocarbons or by hydrogenation of coal or other carbonaceous materials; as well as coal tar products. The presence of aromatics in the treating stock is desirable and in general oils containing less than 20% aromatics respond insufficiently to warrant the expense of the treatment. Depending upon the choice of treating stocks and treating conditions the predominance of certain products of reaction can be varied at will and within wide limits.

Specific applications of the process consist of improving the viscosity index of lubricating oils whose low V. I. is due to the presence of aromatics, or of desulfurization.

In a particular instance, the sulfur content of a kerosene was lowered from 1.6% to .3% and owing to the removal of aromatics the "ring number" had risen from 26 to 53. In order to desulfurize an oil, deficient in aromatics, I may add aromatics to it, prior to introducing acetylene. Gasoline, kerosene, gas oil, etc., can be desulfurized in this manner.

In my preferred procedure I introduce for a prolonged period, which may be of the duration of several hours, acetylene or gases containing acetylene into the oil to be treated, which contains aluminum chloride or other polymerizing catalyst in suspension. During this time the liquid mass is kept agitated to provide for a thorough contact of the reactant. A primary product of reaction is formed, which for some

purposes may form a suitable raw stock for producing my improved hydrocarbon product by ordinary refining methods. Generally, however, I continue the treatment by stopping the influx of acetylene and allowing the mass to digest preferably in an atmosphere of acetylene, and at a moderately elevated temperature, which may be the temperature of the first treatment. The digestion period may extend from  $\frac{1}{2}$  hour to more than 24 hours, depending upon the treating stock and product desired. A secondary product of reaction is formed from which my improved products are separated by known means as explained later.

At times and depending upon the desired end products, acetylenization and digestion periods may be repeated alternately several times. This procedure may prove especially useful in the manufacture of resins.

During the active treatment the temperature is preferably kept below about 50° C., for example between about 30° C. and 50° C.; in some special instances temperatures of 0° C. or even below may be used. For producing high quality products, temperatures above 50° C. should in general be avoided; in some instances temperatures exceeding 50° C., e. g. up to about 100° C., may be applied, for example in cases where the production of somewhat darker reaction products is not objectionable.

During the introduction of acetylene the viscosity of the reaction mass rises and it may become so thick, as to make proper contact with the gas impossible. In such a case the treating stock may be diluted with inert hydrocarbon diluents such as cyclohexane, petroleum ether, kerosene free of aromatics, etc. Should the diluent contain aromatics, then it will participate in the reaction and contribute to the thickening.

The pressure of acetylene can be varied over wide ranges as a general rule. Increase of pressure accelerates the reaction. This may be desirable, when using gases which are relatively poor in acetylene, such as are obtained by cracking or incomplete combustion of hydrocarbons in the electric arc. The acetylene may be applied immediately after its manufacture, whilst still in statu nascendi or at least hot.

The amount of acetylene absorbed, besides being important in the economy of the process, determines to a large extent the nature of the reaction products. Thus the amount of absorbed acetylene may vary from less than about 3% to 10% on the aromatic content of the treating stock

in manufacturing processes in which liquid hydrocarbons are the main products, and from 10% to 20%, when resins are formed. As previously pointed out, stocks containing no or only small percentages of aromatics do not respond readily to acetylenization.

My process is further explained in the attached drawing to which I now refer. Hydrocarbon oil to be treated comprising non-aromatic hydrocarbons and normally containing a substantial portion of aromatic hydrocarbons is admitted to reactor 1 through line 2 from a source not shown. If the oil should be deficient in aromatic hydrocarbons, suitable aromatics may be added through line 3. When the reactor 1 is charged to the desired level, catalyst is introduced through line 4 and acetylene through line 5. Unreacted acetylene or inert gases admixed therewith are vented through line 6 and may be recovered in any suitable manner.

After the reaction has progressed to the desired point, the influx of acetylene is shut off and the reaction mixture is preferably allowed to digest for several hours. Sludge normally containing the spent catalyst settles out and is withdrawn through sludge line 7. Sometimes, however, the reaction mass may become too viscous to allow settling of the sludge. In this case a suitable diluent or precipitant such as liquid propane, petroleum ether, etc., may be added through line 8, which diluent effectively separates sludge and also may separate a portion of substantially all of the resinous reaction products. The entire precipitated mass is then withdrawn through sludge line 7. The supernatant liquid, whose content of aromatics and sulfur compounds, if sulfur compounds were present, has been greatly reduced, is transferred through line 9 to still 10.

After completed acetylenization, one of several courses may be followed, depending on the type of oil treated and the type and amount of diluent used. If the treated oil contains material portions of the high molecular weight reaction products between acetylene, aromatics and sulfur compounds, if sulfur compounds were present, the unreacted portion of the oil which consists essentially of non-aromatic hydrocarbons, is taken overhead together with the diluent, high molecular weight compounds remaining in the still as residue, usually in the form of resins. The latter may be withdrawn through line 11 while the diluent vapors proceed through vapor line 12 and condenser 13, an unreacted oil may be taken as a side stream through line 14 and condenser 15.

If no diluent was used the entire overhead may be conducted through line 14 and condenser 15.

If on the other hand treatment with the diluent was very effective so as to result in the removal of the greater portion of high molecular weight reaction products together with the sludge in reaction vessel 1, then distillation may be required only to distill the diluent, and the refined oil may be withdrawn as still bottoms through line 11.

The product of reaction normally consists of a complicated mixture of many substances, lubricating oils, resins and other viscous hydrocarbons which can be refined or separated by distillation and/or treating with sulfuric acid and/or extraction methods. Inasmuch as aliphatic and naphthenic hydrocarbons are not substantially affected by acetylenization as herein described, the present treating method in combination with distillation affords a means for separating them

from aromatics. After removal of vaporizable constituents, which may include lubricating oils, the residue may be treated with naphtha, petroleum ether, propane and the like, or aromatic hydrocarbons for further fractionation of the resins. Other selective solvents such as B B dichlorethyl ether, nitrobenzene, phenol, cresilic acid, acrolein, furfural, etc., may find suitable applications in many instances.

#### Example I

10

Lubricating stock with a specific gravity of .9640 having a V. I. of -9 was dissolved in petroleum ether. 13.6% aluminum chloride on the weight of the oil were added and dry acetylene was introduced for 3½ hours at 50° C. while agitating. 2.8% acetylene based on the weight of the oil, or approximately 9% based on the aromatics contained therein, were absorbed. The mixture was allowed to digest for 40 minutes at 50° C. and then for 16 hours at room temperature.

The product of reaction was partly solid. It was extracted with petroleum ether (40-60° C. boiling range). The soluble part was filtered through clay and topped; the distillation residue was a lubricating oil amounting to 71.6% of the treating stock and had a good color, a specific gravity of .9338 and a V. I. of 61.

The residue from the first extraction was further extracted with a mixture of benzol and petroleum ether. 12.9% of a brown colored highly viscous mass was recovered after filtering through clay and topping.

The residue from the second extraction was treated with water to decompose the aluminum chloride and its complex compounds and was extracted with benzol. 8.4% of brown resins were obtained after separating benzol from the extract.

#### Example II

40

A cycle stock very rich in aromatics and with a boiling range of about 170° to 340° C. and a specific gravity of 0.9833, obtained in the cracking of mineral oil-containing aromatics, was taken as base material. 3.2% aluminum chloride on the weight of the cycle stock were added and acetylene was introduced for 3 hours at a temperature of 30-31° C. The mass was then allowed to digest for 16 hours at room temperature, after which acetylene was introduced for a further 4 hours at 30-31° C. whilst adding a further amount of 0.6% aluminum chloride. 10.4% acetylene based on the weight of the base material were absorbed.

The very viscous reaction mass was extracted with petroleum ether. The extract, after evaporation of the petroleum ether, was subjected to vacuum distillation and yielded a colourless oil boiling between 50° and 150° C. at 1.2 mm. pressure in a quantity of 26.2% of the base materials, whilst as residue a light brown transparent resin was obtained in a quantity of 7.3% of the base materials.

The residue from the first extraction yielded, on extraction with a mixture of 2 parts petroleum ether and 1 part benzol, an extract from which a light yellow oil fraction boiling between 50 and 140° C. at 1.4 mm. pressure was obtained by vacuum distillation in an amount of 16.6%, and as residue 27.0% of a greenish brown resin.

The residue from the second extraction was treated with water to decompose the aluminium chloride and was extracted with benzol. 22.0% of a brown resin were obtained after evaporation of the solvent.

70

75

76

The total quantity of resins thus amounts to 56.3%, calculated on the base materials.

The oil fractions recovered from the reaction mass can, if desired, be subjected to a new treatment with acetylene, whereby the yield of resins 5 can be increased still further.

While I have found that anhydrous aluminum chloride is the most active catalyst, other catalysts suitable for promoting polymerization reactions 10 can be used as well. To mention a few: boron fluoride, zinc chloride, titanium chloride, ferric chloride, etc. have produced favorable results.

I claim as my invention:

1. In the process of refining a mineral oil containing aromatic and non-aromatic hydrocarbons 15 to produce a refined product having a substantially lower content of aromatic hydrocarbons, the steps of treating said mineral oil with acetylene in the presence of a polymerization catalyst 20 under conditions to react the acetylene with the aromatic hydrocarbons and to convert at least a portion thereof to compounds of higher molecular weights without substantially changing the constitution of the non-aromatic hydrocarbons, 25 and concentrating the unreacted non-aromatic hydrocarbons by separating said higher molecular weight compounds therefrom.

2. The process of claim 22 in which said higher molecular weight hydrocarbons and the remaining substantially unreacted oil are separated 30 by distillation.

3. In the process of refining a mineral lubricating oil containing aromatic hydrocarbons of low viscosity index and non-aromatic hydrocarbons 35 of higher viscosity index to produce a refined lubricating oil of improved viscosity index having a substantially lower content of aromatic hydrocarbons, the steps of treating said mineral lubricating oil with acetylene in the presence of a polymerization catalyst under conditions to react 40 the acetylene with the aromatic hydrocarbons

and to convert at least a portion thereof to resinous compounds of higher molecular weights without substantially changing the constitution of the non-aromatic hydrocarbons, and concentrating the unreacted non-aromatic hydrocarbons by 5 separating said higher molecular weight compounds therefrom.

4. In the process of refining a mineral oil containing aromatic and non-aromatic hydrocarbons and sulfur-bearing compounds to produce a refined product having a substantially lower content of aromatic hydrocarbons and sulfur-bearing compounds, the steps of treating said mineral oil with acetylene in the presence of a polymerization catalyst under conditions to react the 15 acetylene, sulfur-bearing compounds and aromatic hydrocarbons with each other and to convert at least a portion thereof to compounds of higher molecular weights, without substantially changing the constitution of the non-aromatic 20 hydrocarbons, and concentrating the unreacted non-aromatic hydrocarbons by separating said higher molecular weight compounds therefrom.

5. In the process of refining a non-aromatic hydrocarbon oil containing sulfur-bearing compounds to produce a refined product having a substantially lower content of sulfur-bearing compounds, the steps of adding an aromatic hydrocarbon to said oil, treating the resulting mixture with acetylene in the presence of a polymerization catalyst under conditions to react the acetylene, sulfur-bearing compounds and aromatic hydrocarbons with each other and to convert at least a portion thereof to compounds of higher molecular weights, without substantially 35 changing the constitution of the non-aromatic hydrocarbons, and concentrating the unreacted non-aromatic hydrocarbons by separating said higher molecular weight compounds therefrom.

HEIN ISRAEL WATERMAN. 40

CERTIFICATE OF CORRECTION.

Patent No. 2,088,500.

July 27, 1937.

HEIN ISRAEL WATERMAN.

It is hereby certified that error appears in the printed specification of the above numbered patent requiring correction as follows: Page 3, first column, line 28, claim 2, for the claim reference numeral "22" read 1; and that the said Letters Patent should be read with this correction therein that the same may conform to the record of the case in the Patent Office.

Signed and sealed this 19th day of October, A. D. 1937.

(Seal)

Henry Van Arsdale.  
Acting Commissioner of Patents.

The total quantity of resins thus amounts to 56.3%, calculated on the base materials.

The oil fractions recovered from the reaction mass can, if desired, be subjected to a new treatment with acetylene, whereby the yield of resins 5 can be increased still further.

While I have found that anhydrous aluminum chloride is the most active catalyst, other catalysts suitable for promoting polymerization reactions 10 can be used as well. To mention a few: boron fluoride, zinc chloride, titanium chloride, ferric chloride, etc. have produced favorable results.

I claim as my invention:

1. In the process of refining a mineral oil containing aromatic and non-aromatic hydrocarbons 15 to produce a refined product having a substantially lower content of aromatic hydrocarbons, the steps of treating said mineral oil with acetylene in the presence of a polymerization catalyst 20 under conditions to react the acetylene with the aromatic hydrocarbons and to convert at least a portion thereof to compounds of higher molecular weights without substantially changing the constitution of the non-aromatic hydrocarbons, 25 and concentrating the unreacted non-aromatic hydrocarbons by separating said higher molecular weight compounds therefrom.

2. The process of claim 22 in which said higher molecular weight hydrocarbons and the remaining substantially unreacted oil are separated 30 by distillation.

3. In the process of refining a mineral lubricating oil containing aromatic hydrocarbons of low viscosity index and non-aromatic hydrocarbons 35 of higher viscosity index to produce a refined lubricating oil of improved viscosity index having a substantially lower content of aromatic hydrocarbons, the steps of treating said mineral lubricating oil with acetylene in the presence of a polymerization catalyst under conditions to react 40 the acetylene with the aromatic hydrocarbons

and to convert at least a portion thereof to resinous compounds of higher molecular weights without substantially changing the constitution of the non-aromatic hydrocarbons, and concentrating the unreacted non-aromatic hydrocarbons by 5 separating said higher molecular weight compounds therefrom.

4. In the process of refining a mineral oil containing aromatic and non-aromatic hydrocarbons and sulfur-bearing compounds to produce a refined product having a substantially lower content of aromatic hydrocarbons and sulfur-bearing compounds, the steps of treating said mineral oil with acetylene in the presence of a polymerization catalyst under conditions to react the 15 acetylene, sulfur-bearing compounds and aromatic hydrocarbons with each other and to convert at least a portion thereof to compounds of higher molecular weights, without substantially changing the constitution of the non-aromatic 20 hydrocarbons, and concentrating the unreacted non-aromatic hydrocarbons by separating said higher molecular weight compounds therefrom.

5. In the process of refining a non-aromatic hydrocarbon oil containing sulfur-bearing compounds to produce a refined product having a substantially lower content of sulfur-bearing compounds, the steps of adding an aromatic hydrocarbon to said oil, treating the resulting mixture with acetylene in the presence of a polymerization catalyst under conditions to react the acetylene, sulfur-bearing compounds and aromatic hydrocarbons with each other and to convert at least a portion thereof to compounds of higher molecular weights, without substantially 35 changing the constitution of the non-aromatic hydrocarbons, and concentrating the unreacted non-aromatic hydrocarbons by separating said higher molecular weight compounds therefrom.

HEIN ISRAEL WATERMAN. 40

CERTIFICATE OF CORRECTION.

Patent No. 2,088,500.

July 27, 1937.

HEIN ISRAEL WATERMAN.

It is hereby certified that error appears in the printed specification of the above numbered patent requiring correction as follows: Page 3, first column, line 28, claim 2, for the claim reference numeral "22" read 1; and that the said Letters Patent should be read with this correction therein that the same may conform to the record of the case in the Patent Office.

Signed and sealed this 19th day of October, A. D. 1937.

(Seal)

Henry Van Arsdale.  
Acting Commissioner of Patents.

CERTIFICATE OF CORRECTION.

Patent No. 2,088,500.

July 27, 1937.

HEIN ISRAEL WATERMAN.

It is hereby certified that error appears in the printed specification of the above numbered patent requiring correction as follows: Page 3, first column, line 28, claim 2, for the claim reference numeral "22" read 1; and that the said Letters Patent should be read with this correction therein that the same may conform to the record of the case in the Patent Office.

Signed and sealed this 19th day of October, A. D. 1937.

(Seal)

Henry Van Arsdale.  
Acting Commissioner of Patents.